

# UNITED STATES PATENT OFFICE.

FRANK A. FAHRENWALD, OF CLEVELAND, OHIO.

## CHEMICAL WARE OR TECHNICAL APPARATUS AND ALLOYS FOR MAKING SAME.

1,357,550.

Specification of Letters Patent.

Patented Nov. 2, 1920.

No Drawing.

Application filed August 25, 1919. Serial No. 319,821.

To all whom it may concern:

Be it known that I, FRANK A. FAHRENWALD, a citizen of the United States, residing at Cleveland, in the county of Cuyahoga and State of Ohio, have invented a certain new and useful Improvement in Chemical Ware or Technical Apparatus and Alloys for Making Same, of which the following is a full, clear, and exact description.

This invention relates to apparatus for use in the manufacturing chemical industry and has for its object the provision of an inexpensive, chemically resistant alloy for the construction of tanks, valves, pipes, fittings, evaporation pans, stirrers, and the like which shall be sufficiently strong to resist accidental breakage, and also soft enough to permit being machined to shape. All such devices I include under the term "chemical apparatus."

In the production and manipulation of acids, corrosive salts, and some alkalis it is impossible to employ ordinary metals for the parts named because of the contamination of the product and the corrosion of the apparatus. Gold, palladium and platinum are prohibitively expensive; glass and porcelain are subject to breakage as well as being difficult to machine or fit together; and even lead, which is used for some purposes, is mechanically weak. My improved alloy herein described avoids all these difficulties and possesses an extremely high chemical resistivity. My improved alloy consists essentially of chromium, an iron group metal, and a second metal from the chromium group. Carbon and silicon may be present but their quantity should be small since otherwise the alloy will be unduly hard. Tungsten is more resistant chemically than molybdenum when equal atomic proportions are considered, but molybdenum alloys are the more workable and when used in equal weight-percentages the molybdenum has the greater chemical effect owing to its smaller atomic weight which causes the presence of almost twice the number of molecules in a given weight.

For the iron group metal I usually employ iron because of its peculiar availability and its low cost but from a chemical standpoint either nickel or cobalt is superior and of these nickel is the best. Indeed the very best alloy from the chemical standpoint is composed of nickel and tungsten, each of which is the most resistant chemically of

the members of their respective groups, combined with enough chromium to constitute a mutual solvent, but the composition is comparatively expensive and somewhat more difficult to machine. Iron is cheaper than nickel and with molybdenum and chromium forms an alloy which is sufficiently resistant for almost all uses, as well as one which is comparatively easy to work.

The carbon and silicon have no beneficial function but are present as impurities. They are not obnoxious if their proportion be low, say less than about 1%. Certain typical formulas are as follows, the proportions being by weight:

|                             | A            | B  | C  | D       |    |
|-----------------------------|--------------|----|----|---------|----|
| Chromium .....              | 60           | 55 | 60 | (40-60) | 75 |
| Iron group metals .....     | 20           | 25 | 30 | (10-40) |    |
| Molybdenum like metal ..... | 20           | 20 | 10 | (10-20) |    |
| Carbon .....                | Less than 1% |    |    |         |    |
| Silicon .....               | Less than 1% |    |    |         |    |

Column A gives the alloy that appears to be the most resistant chemically of any I have investigated. Columns B and C give the compositions which are most easily made when the iron group metal employed is iron. Column D indicates the limits of favorable composition.

The alloys can be made in any convenient manner and no especial precautions are necessary except to keep the carbon and silicon low. Thus any of the alloys can be made by melting the pure ingredients in an electric or other furnace out of contact with carbon. Owing to the fact that chromium generally occurs in connection with iron as in chromite ore,  $(FeCr_2O_4)$  it is most conveniently obtained in the form of ferro chrome, which is an alloy of approximately iron 34.5 and chromium 65.5, along with small quantities of carbon and silicon. If suitable precautions are observed in the reduction, such as the employment of the alumino-thermic process or that process explained in my application filed July 13, 1920 Ser. No. 1,346,187, the presence of carbon and silicon can be almost entirely avoided, and in fact by other known methods these can be brought sufficiently low to produce a workable alloy. It is merely necessary to add metallic tungsten or molybdenum to such molten ferro-chrome to produce the alloys shown in columns B and C, and for this reason I esteem these most highly, notwithstanding the greater resistiv-

ity of the nickel alloy. I do not restrict myself to such a small proportion of carbon and silicon as shown in the preferred example, since somewhat larger quantities 5 will not interfere with the use of the alloy for most purposes, and such alloys can be made more cheaply.

It will be understood that other ingredients may be added within the scope of 10 my invention and that changes may be made within the scope and purview of my claims. It will also be understood that I do not confine myself to the use of only one iron group metal or only one molybdenum like 15 metal in my improved alloy.

Having thus described my invention what I claim is:—

1. An alloy for the purpose described containing 40% to 60% of chromium together 20 with 10% to 20% of one or more other metals of the chromium group, the balance consisting principally of one or more iron group metals.

2. An alloy for the purpose described consisting essentially of ferro-chrome with the addition of ten to twenty per cent. of molybdenum-like metal.

3. An alloy for the purpose described, containing a preponderance of chromium, an 30 iron group metal, and at least ten per cent. of a second metal from the chromium group.

4. An alloy for the purpose described containing a preponderance of chromium, and at least ten per cent. each of a metal or 35 metals from the iron group and of another metal or metals from the chromium group.

5. Chemical apparatus made of an alloy containing 40 to 60 per cent. of chromium, together with 10 to 20 per cent. of one or 40 more other metals of the chromium group, and 10 to 20 per cent. of one or more metals from the iron group.

6. Chemical apparatus made of an alloy consisting essentially of ferro-chrome with 45 the addition of ten to twenty per cent. of a molybdenum-like metal.

7. Chemical apparatus made of an alloy containing an iron group metal combined with at least an equal amount of chromium and at least ten per cent. of one or more 50 other metals of the chromium group.

8. Chemical apparatus made of an alloy containing chromium, at least ten per cent. of another metal from the chromium group, and an iron group metal, chromium being 55 present in a proportion at least as great as any other ingredient.

9. Chemical apparatus made of an alloy containing a preponderance of chromium, an iron group metal, and at least ten per cent. 60 of a second metal from the chromium group.

10. Chemical apparatus made of an alloy containing chromium, iron, and a molybdenum-like metal, each of the last two being present to a proportion of at least about ten 65 per cent., and the chromium being present to a proportion at least as great as either of the other metals.

11. The process of making a chemically 70 resistant metallic alloy which contains the steps of first reducing chromite ore and second adding from ten to twenty per cent. of a molybdenum like metal to the molten product of such reduction.

12. An alloy for the purpose described 75 containing nickel, chromium, and tungsten, chromium being preponderant and tungsten being present to a proportion of at least five per cent.

13. An alloy for the purpose described 80 consisting of from ten to twenty per cent. each of nickel and a tungsten-like metal, together with an amount of chromium equal to at least about 40% of the whole.

14. Chemical apparatus made of an alloy 85 of nickel, chromium, and at least about five per cent. of a tungsten-like metal, chromium being preponderant.

In testimony whereof I hereunto affix my signature.

FRANK A. FAHRENWALD.